

Feb. 7, 1933.

A. DECHENNE

1,896,704

PROCESS FOR MANUFACTURING STEEL TIRES AND  
THE LIKE BY FORGING AND PRESSING INGOTS

Filed March 13, 1931

*Fig. 1.*



*Fig. 2.*



*Fig. 3.*



*Fig. 4.*



## UNITED STATES PATENT OFFICE

ALBERT DECHENNE, OF SEBAIN, BELGIUM

## PROCESS FOR MANUFACTURING STEEL TIRES AND THE LIKE BY FORGING AND PRESSING INGOTS

Application filed March 13, 1931, Serial No. 522,333, and in Belgium March 22, 1930.

The object of the present invention is an improvement in the process of manufacturing steel tires, rims, bands, hoops and flanges for wheels, by forging and pressing ingots.

- 5 It is a matter of fact that ingots have a dead head containing the segregations and impurities of the block, and of course the material of said dead head must be eliminated and cannot be used for manufacturing such 10 steel tires, rims, bands, hoops and flanges, because such articles can only be manufactured with sound material.

Now, it is very difficult to eliminate just the segregation zone of the ingot and manifold 15 processes have already been proposed either to cut away or to eliminate said dead head. All processes hitherto known are very complicated and require manifold manipulations.

Now, the new process according to the invention 20 enables in a very simple manner to create a torus-shaped body containing only sound, material and apt to be worked for obtaining the finished steel, tire, rim, band, hoop, flange or the like.

25 The main characteristics of said process consist in placing an ingot with its dead head down on a cavity of an anvil, flattening said ingot and simultaneously driving said dead head into the cavity of the anvil, thus obtaining a flat workpiece. Then the flattening procedure is stopped, the workpiece is lifted up and a ring-die or bed-die is intercalated between said workpiece and said anvil, whereupon a mandrel is placed on the central part of said workpiece. Then the hammering or forging action or pressing is continued so as to expel said central part of the workpiece by means of said mandrel, the latter passing entirely through the workpiece, so that the central part falls out of same.

Obviously the punching can be started by means of the mandrel alone before inserting the ring-die.

45 The new process will be described in detail hereafter with reference to the diagrammatic figures of the accompanying drawing, showing the various phases of the manufacturing process.

50 Fig. 1 is a diagrammatic view in cross sec-

tion of the hammer of a press and of the corresponding anvil with an ingot between them;

Fig. 2 is a similar view showing a second phase;

Fig. 3 shows the workpiece in a third phase 55 with the hammer and the anvil in a similar view as shown in Fig. 1 after insertion of a mandrel between workpiece and hammer;

Fig. 4 shows the finished workpiece.

In these figures, the head of the hammer is 60 designed by reference numeral 1 and the anvil by numeral 7, both being shown in vertical axial cross section. The anvil has a semi-spherical central cavity 15, whilst the hammer face 12 has in its center a small cavity 65 9 for the purpose indicated in the following description.

On executing the process of manufacturing steel tires, the truncated cone-shaped ingot 11, heated to a sufficient temperature 70 appropriate for swaging, is brought perpendicularly under the hammer 1 or hammer face 12 or under the head of the forging press (Fig. 1), the dead head of said ingot resting on the semi-spherical cavity 15 of the 75 matrix or anvil 7.

The dead head of the ingot contains the segregations and impurities to be eliminated in the manufacture of tires, hoops and the like.

By hammering the ingot, the dead head containing the before-mentioned segregations and impurities enters into the semi-spherical cavity 15 of the matrix or mould 7 and takes the shape of this cavity. On continuing the hammering action, the sound portion of the ingot will be extended over the plane surface of the mould or anvil. The semi-spherical cavity 15 of the matrix 7 serves also to hold fast the dead head of the ingot and to bound it, so that the dead head does not enter into the sound material, the latter building up the torus-shaped workpiece 3 (Fig. 2).

As can be seen from said Fig. 2, the workpiece is now provided with an excrescence 5 having a shape according to the cavity 15, i. e. in the present case a semi-spherical shape. The cavity 15 has a capacity or volume able to contain 15 to 20% of the ingot 11, as gen- 100

erally in normally cast ingots the segregations and impurities have a volume of 15 to 20% of the whole ingot and are together in the dead head of the ingot.

5 During the flattening process, the hammering has produced on the upper surface of the workpiece a small bubble 10 just in its center, according to the central cavity 9 of the hammer face 12. On the upper face of 10 the workpiece a truncated mandrel 2 is placed, its position being fixed by said bubble 10, because said mandrel has a corresponding cavity 14 in its base, and has also a small centering bubble 13 corresponding to 15 the cavity 9 of the hammer face 12 (Fig. 4). On continuing forging or pressing, said mandrel 2 is driven into the central part of the workpiece 3 and so the sound material of the central part will be driven sideways.

20 The pressing or forging process is interrupted and a ring die 4 is inserted between the workpiece 3 and the anvil 7 and an auxiliary head piece 8 of cylindrical shape is placed on the top of the mandrel 2. This head piece 25 8 has in its base also a small semi-spherical cavity 13, corresponding to the bubble on the top of the mandrel 2 and has also a top bubble corresponding with the cavity 9 of the head face of the hammer 1.

30 Now the forging or pressing process is continued for entirely expelling the central part of the workpiece, as can be seen from Fig. 4, where this central part lays in the 35 semi-spherical cavity 15 of the anvil 7 and is entirely separated from the torus-shaped workpiece 32, the latter containing only sound material. The workpiece 32 with its central hole is now brought under another 40 anvil for being forged there and afterwards it will be heated again, if necessary, and will be drawn out in the usual manner.

After having rolled to rings, the latter may be cut into sections and said sections 45 stretched for making bars thereof which can be used for any purpose whatever.

For automatically centering the mandrel 2, the small cavity 9 is provided in the hammer face 12, so that this small cavity 9 creates in the axis of the workpiece the small projection or bubble 10 and as the base of 50 the mandrel 2 possesses a corresponding small cavity 14, the centering of the mandrel is automatically obtained, and so it will be sure that only the central part of the workpiece, containing all segregations and 55 impurities, that is to say the central part corresponding to the dead head of the ingot will be driven out, expelled and separated from 60 the sound part of the workpiece.

Furthermore, experience has shown that on putting the ingot with its dead end on the semi-spherical cavity 15 of the anvil 7, only the lost head of the ingot penetrates into said 65 cavity, whilst the sound material will be

spread out during the forging, pressing or hammering action round this cavity 15.

I claim:

1. In a process of manufacturing steel tires and the like by forging and pressing to ingots, the steps of placing an ingot with its dead head in a cavity of an anvil, said cavity having a volume capable of receiving the complete piping and segregation part, flattening said ingot and simultaneously driving the dead head completely into said cavity, thus obtaining a flat workpiece having a central projection on the face formed by the piping and segregation part of the ingot, and punching out the central part of the workpiece together with said projecting portion.

2. In a process of manufacturing steel tires and the like by forging and pressing ingots, the steps of placing an ingot with its dead head in a hemispherical cavity of an anvil, said cavity having a volume to completely receive the piping and segregation zone; flattening said ingot and simultaneously driving the dead head completely into said cavity so as to form a hemispherical projection, forming a centering projection on the face of the workpiece, and punching out the central part of the workpiece together with the projecting dead head.

In testimony whereof I signed hereunto my name.

ALBERT DECHENNE.

100

105

110

115

120

125

130